

Patented May 29, 1945

2,377,129

# UNITED STATES PATENT OFFICE

2,377,129

## FLOTATION OF PHOSPHATE MINERALS

Ludwig J. Christmann, Yonkers, N. Y., and Stephen E. Erickson, Calumet, Minn., assignors to American Cyanamid Company, New York, N. Y., a corporation of Maine

No Drawing. Original application June 20, 1940. Serial No. 341,438. Divided and this application June 5, 1943, Serial No. 489,814

10 Claims. (Cl. 209—166)

The present invention relates to the froth flotation of phosphate minerals and more specifically relates to a method of improving the promoting power of the promoters ordinarily employed in concentrating phosphate ore values by froth flotation. This application is a division of our co-pending application Serial No. 341,438 filed June 20, 1940.

It is well known in the art that the values of phosphate ores can be concentrated or recovered by froth flotation processes in which fatty acid substances are employed as promoters. Among the more important promoters used heretofore are the free fatty acids themselves such as oleic acid, fish oil fatty acids, talloel, fatty acid soaps, and the like. In carrying out the actual froth flotation operation these various promoters may be mixed with an alkali such as caustic soda along with a water-immiscible oil such as fuel oil and may or may not also contain a frother such as pine oil or kerosene. While such phosphate recovery processes have been employed successfully on a commercial basis they are not entirely satisfactory in that it is difficult to obtain a phosphate concentrate having a low percentage of insoluble material. The value of the phosphate concentrate is very largely determined by the amount of insoluble material which is present and it is therefore very desirable that a phosphate concentrating process be developed which would result in the production of a lower insoluble containing concentrate.

In accordance with the present invention it has been discovered that the promoting power of the fatty acid type promoters employed in concentrating phosphate materials by froth flotation can very greatly be increased by adding a low percentage of an aliphatic alcohol or aliphatic ether alcohol to the promoter prior to the froth flotation operation. Some of the prior processes have used alcoholic solutions of flotation reagents, e. g., where the alcohol used is equal to or greater than the amount of flotation reagent. In such processes the alcohol was used as a solvent for the flotation reagents and was merely a method of obtaining the flotation reagents in highly concentrated form. In the present invention, however, the fatty acid type flotation reagent is diluted with about 20% or less of an alcohol to increase the promoting power. The quantity of alcohol employed in carrying out the present invention is very much less than the quantities employed as solvents in the prior solution methods. The exact reason why the promoting power of the phosphate flotation promoters is increased by the diluting with a small amount of an alcohol has not been definitely determined and we do not desire therefore to limit the present invention to any theory or explanation as to why the promoting power is increased.

In connection with the recovery of values from phosphate ores on a commercial scale we have found that we can reduce the percentage of insolubles in the concentrate on an average of about one to two percent when compared to the ordinary fatty acid flotation process, while at the same time the reagent cost is increased only about one cent per ton of phosphate concentrate, and hence, the present invention results in a very economical saving in the concentration of phosphate ores. The higher grade concentrate will also bring a better price as a 1% increase in grade is equivalent to about fifteen cents increase in value per ton of concentrate.

15 In carrying out the present invention the fatty acid promoter is diluted with about 20% or less of an aliphatic alcohol or aliphatic ether alcohol. This mixture is then employed in the usual manner for conducting the froth flotation. We may, however, mix the fatty acid alcohol mixture with an equal quantity of fuel oil and then add this 50/50 mixture to the flotation feed or pulp containing the correct quantity of caustic and then condition for a short time prior to the froth flotation.

20 It is an advantage of the present invention that the promoting power of the fatty acid type promoters are increased by diluting with 20% or less of any of the well known aliphatic alcohols or ether alcohols and is not limited to any particular alcohol or ether alcohol. Among the aliphatic alcohols that have been found to be useful are those such as methyl, ethyl, propyl, iso-propyl, butyl, iso-butyl, octyl; the polyhydroxy alcohols such as glycol, diethylene glycol, or polyethylene 25 glycols, and the various ether alcohols such as mono-methyl ether of diethylene glycol, mono-ethyl ether of diethylene glycol, mono-butyl ether of diethylene glycol and the like. The term "aliphatic alcohol" as used in the appended claims is intended to include the unsubstituted mono- and poly-hydric aliphatic alcohols and the aliphatic ether alcohols such as those listed above.

30 The invention will be further illustrated in connection with the following specific examples.

### EXAMPLE 1

#### Tests on phosphate ore

35 The ore sample used in these flotation tests is from the Brewster, Florida, region, and is a representation deslimed flotation feed.

40 In running the flotation tests, a charge of the phosphate rock, containing 600 grams of dry solids was employed for each test. Sufficient water was added to give a pulp density of 72% solids. The resultant pulp was agitated by means of a mechanical-type mixer. Reagents were added in quantities as shown in the descriptions for the 45 individual tests (Table 1) and the pulp was then

agitated for four minutes. Each of the reagent mixtures tested was made up as a 50% solution in light fuel oil before adding it to the flotation pulp.

After agitation the pulp was transferred to a laboratory-size Fagergren flotation machine and diluted to 22% solids with water. Air was then admitted to the cell and a rougher concentrate was skimmed off for a period of one and a half minutes. This product was replaced in the flotation machine, without additional reagents, and a cleaner concentrate removed by flotation for a period of one minute.

The metallurgical results obtained in these tests are tabulated in Table 1.

contained 9.4% isopropyl alcohol and 90.6% talloel.

Tests were run on two different day shifts. The results of these tests are given below:

### First day

| Section | Feed                 |           | Concentrate          |                  | Promoter                    |
|---------|----------------------|-----------|----------------------|------------------|-----------------------------|
|         | Per cent<br>B. P. L. | Tons/hour | Per cent<br>B. P. L. | Percent<br>insol |                             |
| East    | 39.11                | 53.03     | 72.21                | 7.20             | Talloel.                    |
| West    | 39.00                | 54.51     | 73.65                | 4.75             | Talloel-alcohol<br>mixture. |

15

TABLE I  
Metallurgical data

| Test No. | Feed, percent B. P. L. | Cleaner concentrate |                  |                |                | Cleaner tailing |                  |                |             | Rougher tailing  |                |                 |                      | Mixture tested       |                      |                      |      | Promoter, lbs./ton of<br>feed |
|----------|------------------------|---------------------|------------------|----------------|----------------|-----------------|------------------|----------------|-------------|------------------|----------------|-----------------|----------------------|----------------------|----------------------|----------------------|------|-------------------------------|
|          |                        | Percent wt.         | Percent B. P. L. | Percent insol. | Dist. B. P. L. | Percent wt.     | Percent B. P. L. | Dist. B. P. L. | Percent wt. | Percent B. P. L. | Dist. B. P. L. | Percent wt.     | Percent B. P. L.     | Dist. B. P. L.       | Promoter             | Diluent              |      |                               |
|          |                        |                     |                  |                |                |                 |                  |                |             |                  |                |                 |                      |                      |                      |                      |      |                               |
| 1        | 32.91                  | 28.98               | 74.41            | 4.47           | 65.48          | 5.22            | 53.48            | 8.48           | 65.82       | 13.02            | 26.04          | Talloel H.....  | None.....            | None.....            | None.....            | None.....            | 1.00 |                               |
| 2        | 32.96                  | 28.84               | 76.32            | 3.73           | 66.78          | 6.65            | 59.30            | 11.96          | 64.51       | 10.86            | 21.26          | Talloel H.....  | None.....            | None.....            | None.....            | None.....            | 0.74 |                               |
| 3        | 32.23                  | 37.60               | 74.58            | 5.56           | 84.40          | 2.97            | 38.31            | 3.42           | 59.43       | 6.81             | 12.18          | Talloel H—91%   | Ethyl alcohol—9%     | Ethyl alcohol—9%     | Ethyl alcohol—9%     | Ethyl alcohol—9%     | 1.06 |                               |
| 4        | 32.70                  | 36.07               | 74.75            | 5.19           | 80.01          | 4.47            | 58.65            | 7.78           | 59.46       | 6.92             | 12.21          | Talloel H—91%   | Talloel H—91%        | Talloel H—91%        | Talloel H—91%        | Talloel H—91%        | 0.78 |                               |
| 5        | 33.03                  | 34.99               | 75.09            | 3.99           | 79.55          | 3.96            | 50.93            | 6.11           | 61.05       | 7.76             | 14.34          | Talloel H—91%   | Isopropyl alcohol—9% | Isopropyl alcohol—9% | Isopropyl alcohol—9% | Isopropyl alcohol—9% | 1.00 |                               |
| 6        | 32.70                  | 32.34               | 75.43            | 3.92           | 74.60          | 3.92            | 49.83            | 5.97           | 63.74       | 9.97             | 19.43          | Talloel H—91%   | Talloel H—91%        | Talloel H—91%        | Talloel H—91%        | Talloel H—91%        | 0.75 |                               |
| 7        | 33.34                  | 33.66               | 75.26            | 5.12           | 75.97          | 4.97            | 48.22            | 7.19           | 61.37       | 9.15             | 16.84          | Talloel H—91%   | Methyl alcohol—9%    | Methyl alcohol—9%    | Methyl alcohol—9%    | Methyl alcohol—9%    | 0.99 |                               |
| 8        | 32.63                  | 29.81               | 76.38            | 3.76           | 69.76          | 4.57            | 53.05            | 7.33           | 65.62       | 11.39            | 22.91          | Talloel H—91%   | Talloel H—91%        | Talloel H—91%        | Talloel H—91%        | Talloel H—91%        | 0.75 |                               |
| 9        | 33.02                  | 28.60               | 76.53            | 3.32           | 66.05          | 5.16            | 54.24            | 8.48           | 66.34       | 12.68            | 25.47          | F. O. F. A..... | None.....            | None.....            | None.....            | None.....            | 0.99 |                               |
| 10       | 32.78                  | 22.89               | 76.95            | 3.05           | 53.73          | 4.00            | 58.22            | 7.11           | 73.11       | 17.56            | 39.16          | F. O. F. A..... | None.....            | None.....            | None.....            | None.....            | 0.75 |                               |
| 11       | 32.92                  | 32.35               | 76.61            | 3.27           | 75.28          | 5.36            | 53.31            | 8.68           | 62.29       | 8.48             | 16.04          | F. O. F. A.—91% | Ethyl alcohol—9%     | Ethyl alcohol—9%     | Ethyl alcohol—9%     | Ethyl alcohol—9%     | 1.00 |                               |
| 12       | 32.74                  | 29.48               | 76.28            | 3.38           | 68.69          | 4.14            | 55.17            | 6.98           | 66.38       | 12.00            | 24.33          | F. O. F. A.—91% | Ethyl alcohol—9%     | Ethyl alcohol—9%     | Ethyl alcohol—9%     | Ethyl alcohol—9%     | 0.76 |                               |
| 13       | 32.71                  | 22.36               | 75.74            | 3.49           | 51.77          | 7.22            | 62.95            | 13.89          | 70.42       | 15.95            | 34.34          | Talloel L.....  | None.....            | None.....            | None.....            | None.....            | 0.71 |                               |
| 14       | 32.87                  | 29.42               | 76.10            | 3.76           | 68.12          | 5.06            | 66.10            | 8.64           | 65.52       | 11.66            | 23.24          | Talloel L—91%   | Ethyl alcohol—9%     | Ethyl alcohol—9%     | Ethyl alcohol—9%     | Ethyl alcohol—9%     | 0.75 |                               |
| 15       | 32.35                  | 27.42               | 75.85            | 3.37           | 64.29          | 5.59            | 57.97            | 10.01          | 66.99       | 12.41            | 25.70          | Talloel L—91%   | Isopropyl alcohol—9% | Isopropyl alcohol—9% | Isopropyl alcohol—9% | Isopropyl alcohol—9% | 0.75 |                               |
| 16       | 32.24                  | 33.02               | 73.73            | 4.42           | 73.22          | 5.69            | 53.31            | 9.13           | 61.29       | 9.57             | 17.64          | Talloel L.....  | None.....            | None.....            | None.....            | None.....            | 1.14 |                               |
| 17       | 32.88                  | 32.51               | 76.02            | 3.95           | 75.18          | 4.24            | 56.02            | 7.22           | 63.25       | 9.15             | 17.60          | Talloel L—91%   | Ethyl alcohol—9%     | Ethyl alcohol—9%     | Ethyl alcohol—9%     | Ethyl alcohol—9%     | 0.99 |                               |
| 18       | 32.88                  | 32.31               | 75.26            | 3.97           | 73.95          | 4.37            | 50.68            | 6.74           | 63.32       | 10.03            | 19.31          | Talloel L—91%   | Isopropyl alcohol—9% | Isopropyl alcohol—9% | Isopropyl alcohol—9% | Isopropyl alcohol—9% | 0.99 |                               |
| 19       | 32.79                  | 30.15               | 75.77            | 3.98           | 68.67          | 5.96            | 53.48            | 9.72           | 63.89       | 10.58            | 20.61          | Talloel C.....  | None.....            | None.....            | None.....            | None.....            | 0.74 |                               |
| 20       | 32.99                  | 34.91               | 75.09            | 4.58           | 70.46          | 4.41            | 48.65            | 6.50           | 60.68       | 7.63             | 14.04          | Talloel C.....  | None.....            | None.....            | None.....            | None.....            | 0.99 |                               |
| 21       | 33.11                  | 31.36               | 77.18            | 3.92           | 73.09          | 4.45            | 53.65            | 7.21           | 64.19       | 10.16            | 19.70          | Talloel L—91%   | Ethyl alcohol—9%     | Ethyl alcohol—9%     | Ethyl alcohol—9%     | Ethyl alcohol—9%     | 0.75 |                               |
| 22       | 33.88                  | 37.76               | 75.98            | 5.19           | 84.89          | 4.59            | 39.66            | 5.37           | 57.65       | 5.84             | 9.94           | Talloel L—91%   | Ethyl alcohol—9%     | Ethyl alcohol—9%     | Ethyl alcohol—9%     | Ethyl alcohol—9%     | 0.99 |                               |

The reagents kept constant in the above tests were:

Lbs./ton  
0.75  
4.00

Caustic soda.....

Fuel oil (total).....

F. O. F. A. designates fish oil fatty acid. Talloel H, L & C designates talloel acid from three different sources.

### EXAMPLE 2

50

### Second day

| Section | Feed                 |           | Concentrate          |                  | Promoter                    |
|---------|----------------------|-----------|----------------------|------------------|-----------------------------|
|         | Per cent<br>B. P. L. | Tons/hour | Per cent<br>B. P. L. | Percent<br>insol |                             |
| 55      | 39.64                | 48.62     | 73.77                | 5.30             | Talloel.                    |
|         | 41.10                | 50.88     | 74.64                | 4.45             | Talloel-alcohol<br>mixture. |

60

A third test was run on another day under slightly different conditions. The results are given in Table III.

TABLE III

| Section | Feed     |        | Concentrate |        |        | Tails,<br>B. P. L. | Ratio | Recov. | Lbs./ton conc. |         |      |         |
|---------|----------|--------|-------------|--------|--------|--------------------|-------|--------|----------------|---------|------|---------|
|         | B. P. L. | T./hr. | B. P. L.    | Insol. | T./hr. |                    |       |        | Fuel oil       | Talloel | NaOH | Alcohol |
| East    | 40.39    | 47.45  | 73.65       | 5.80   | 22.92  | 9.18               | 2.07  | 88.1   | 14.39          | 2.32    | 0.86 | 0.21    |
| West    | 40.05    | 48.31  | 74.40       | 5.35   | 23.23  | 8.26               | 2.08  | 89.3   | 15.49          | 1.99    | 0.80 |         |

In the above test the conditions were as follows:

Test duration—5 hours (6:00 p. m.—11:00 p. m.)  
16 gallons isopropyl alcohol and 20 gallons fuel oil added to 255 gallons 50/50 mixture talloel and fuel oil. This mixture used on west section in place of regular 50/50 mixture of talloel and fuel oil.

What we claim is:

1. In the recovery of values from phosphate rock by froth flotation, the process which comprises subjecting an aqueous pulp of phosphate rock to froth flotation in the presence of a fish oil fatty acid diluted with about 10% of ethyl alcohol as the flotation promoter.
2. In the recovery of values from phosphate rock by froth flotation, the process which comprises carrying the flotation out in the presence of a fish oil fatty acid diluted with about 10% of an aliphatic alcohol.
3. The improvement in the recovery of phosphate rock values by froth flotation, processes which comprise subjecting an aqueous pulp of phosphate rock to froth flotation in the presence of a phosphate rock ore promoter of the group consisting of higher fatty acids, mixtures of higher fatty acids, and soaps of such acids, said promoters being diluted with at least one aliphatic alcohol, the alcoholic content of said promoter being from about 9% to not more than about 20%.
4. In the recovery of values from phosphate rock by froth flotation, the process which comprises subjecting an aqueous pulp of phosphate rock to froth flotation in the presence of a fish oil fatty acid diluted with from about 9% to not more than about 20% of an aliphatic alcohol.
5. In the recovery of values from phosphate rock by froth flotation, the process which comprises subjecting an aqueous pulp of phosphate rock to froth flotation in the presence of talcoel
6. In the recovery of values from phosphate rock by froth flotation, the process which comprises subjecting an aqueous pulp of phosphate rock to froth flotation in the presence of talcoel diluted with about 10% of an aliphatic alcohol.
7. In the recovery of values from phosphate rock by froth flotation, the process which comprises subjecting an aqueous pulp of phosphate rock to froth flotation in the presence of talcoel diluted with about 10% of ethyl alcohol.
8. In the recovery of values from phosphate rock by froth flotation, the process which comprises subjecting an aqueous pulp of phosphate rock to froth flotation in the presence of oleic acid diluted with from about 9% to not more than about 20% of an aliphatic alcohol.
9. In the recovery of values from phosphate rock by froth flotation, the process which comprises subjecting an aqueous pulp of phosphate rock to froth flotation in the presence of oleic acid diluted with about 10% of an aliphatic alcohol.
10. In the recovery of values from phosphate rock by froth flotation, the process which comprises subjecting an aqueous pulp of phosphate rock to froth flotation in the presence of oleic acid diluted with about 10% of ethyl alcohol.

LUDWIG J. CHRISTMANN.  
STEPHEN E. ERICKSON.